

Sept. 28, 1948.

O. J. NELSON

2,450,013

APPARATUS FOR PRODUCING ROCK WOOL

Filed May 5, 1943

2 Sheets-Sheet 1



INVENTOR:  
OLIVER J. NELSON,

BY *John H. Cassidy*,  
HIS ATTORNEY.

Sept. 28, 1948.

O. J. NELSON

2,450,013

APPARATUS FOR PRODUCING ROCK WOOL

Filed May 5, 1943

2 Sheets-Sheet 2



INVENTOR:  
OLIVER J. NELSON,

By *John H. Cassidy*,  
HIS ATTORNEY.

## UNITED STATES PATENT OFFICE

2,450,013

## APPARATUS FOR PRODUCING ROCK WOOL

Oliver J. Nelson, Parsons, Kans., assignor to  
himself as trustee

Application May 5, 1943, Serial No. 485,715

15 Claims. (Cl. 263—27)

**1**  
This invention relates to apparatus for producing molten slag for use in rock or mineral wool. It does not, however, contemplate the use of novel means for blowing the slag, its novelty being confined to means for melting and heat conditioning the material preparatory to blowing.

The general object of the invention is to provide means for efficiently producing in a facile manner molten slag in a uniform condition suitable for blowing.

A specific object of the invention is to provide apparatus employing a cupola and a method whereby such a slag may be produced by gas firing. Heretofore a cupola has been used for the production of slag but only when a solid fuel, coke, was used, the fuel being mixed with the rock before or as the cupola was charged. The use of a gaseous or liquid fuel has been proposed but no instance is known where success has attended any prior attempts to use this type of fuel. The presence in some localities of large supplies of natural gas makes such a procedure desirable.

While the novelty of the invention is defined in the appended claims, it may be stated broadly that success of the apparatus has been obtained primarily by an arrangement in which an upper wall or arch is spaced above a lower wall or weir leaving a space for the continuous flow of molten material over the weir, with a flame directed into the cupola approximately from this space; all arranged in such a manner that the slag bleeds off without blocking the opening.

The results have been obtained by the use of surface combustion. A combustible mixture of fuel and air are expelled from the burners positioned at or proximate the exit, so that they are projected upon the surrounding rock which forms a mantle therefor.

The exit from the cupola leads to a forehearth in which further heat is applied and where that heat can be closely regulated to produce a slag of the exact consistency required.

Other novel arrangements are present, such as the introduction of the combustible mixture through the upper wall, or arch, which is water cooled, so that the fuel may be mixed with air before introduction to the burners.

Fig. 1 is a top plan view of a cupola or a furnace embodying this invention;

Fig. 2 is a front elevational view;

Fig. 3 is a side elevational view;

Fig. 4 is a section on line 4—4, Fig. 3;

Fig. 5 is a section on line 5—5, Fig. 2; and

Fig. 6 is a section on line 6—6, Fig. 3.

The furnace includes a cupola and a forehearth. The furnace has side walls 1 and a rear

**2**  
wall 2, constructed of spaced metal plates forming a water jacket. These walls extend upwardly from the base of the furnace a distance, in a typical installation, of eight feet. Above these walls there is a hood 3, constructed preferably of sheet metal and leading to a stack 4. Charging doors 5 are positioned in the front of the hood 3.

The front wall of the cupola is water cooled and has a top vertical section 6, but with the inner plate of this vertical section connected to an inclined plate 7 forming an inclined wall above the outlet of the cupola. The lower end of this front wall forms an arch 8 which is spaced above a bottom water cooled wall or weir 9, thus forming a slot or opening 10 which communicates with the forehearth. The bottom of the cupola has a dump door 11.

The forehearth has masonry side walls 12, masonry arch or roof 13, and front wall 14. The weir 9 rests against a masonry wall 15 in the forehearth. The walls of the forehearth are surrounded by a water jacket. Slag notches 16 are positioned in the front of the forehearth, through which the molten slag is discharged for blowing. The bottom of the forehearth is provided with dump doors 17.

The dump doors 11 and 17 are covered with a fill composed preferably of six inches of mineral wool 18 placed directly on top of the doors, and three inches of earth 19 on top of the mineral wool. This earth may be clay or soil existing at the plant location.

The weir 9 is inclined forwardly from top to bottom at an angle of approximately 60°, while the slope of the upper wall 7 is approximately 45°. The burners 30 are directed downwardly and inwardly in such a way, and in such proximity, that the opening 10 is in a very hot zone.

The water jacket of the walls is connected with the weir 9 as well as with the inclined upper front wall so that the entire system is interconnected and may be served by a water inlet 20 and an outlet 21. The heated water, or as much as is needed, may be used for boiler water to produce steam for blowing, and the remaining portion may be cooled by means of a spray pond. A pump for circulating the water and the spray pond are not shown, such means being well understood in the art.

A mixture of combustible gas, such as natural gas, and air is supplied to the burners 30 through a manifold 22. This manifold is positioned inside the arch 8, where it is cooled by the water in the jacket, thus protecting it from pre-ignition.

Heat for the forehearth is supplied by a plurality of burners 23 projecting downwardly from the top wall or arch 13 of the forehearth, and are supplied from a manifold 24. Where it is desirable to eliminate some undesirable compounds, especially sulphur compounds, from the rock, an oxidizing flame may be employed by introducing an excess of air in the fuel mixture.

In the forehearth the bottom of the slag notches 16 is slightly above the bottom of the forehearth, formed by the earthen layer 19, so that a body of molten slag is kept in the forehearth. This gives a better opportunity for controlling the viscosity of the slag at the outlet. An additional result is obtained by this arrangement, where the cupola is charged with more than one kind of material. Sometimes it is necessary to use a mixture of two or more kinds of material to make a satisfactory wool, or a particular type of wool. In such a case if a pool of molten material is maintained in the forehearth, the different materials have a time period for soaking and combining together before flowing through the outlet to the blowing nozzle.

The furnace may be supported in any convenient manner. Preferably it is positioned on I-beams beneath the walls, the I-beams being supported by pillars sufficiently above the floor to give satisfactory working conditions under the furnace for cleaning it out.

The following is, by way of illustration, a chemical analysis of a typical rock which has been used and found satisfactory in the operation of the apparatus:

|                    |        |
|--------------------|--------|
| Calcium oxide      | 26.00  |
| Iron alumina oxide | 7.21   |
| Silicon dioxide    | 45.55  |
| Magnesium dioxide  | .47    |
| Sulphur trioxide   | .41    |
| Carbon dioxide     | 20.36  |
|                    | 100.00 |

The rock charged to the cupola is of a size from one to four inches, with a normal amount of fine material left from crushing and screening. The rock is charged to the cupola through the doors 5 in such a way that the sides are kept considerably higher than the center. This tends to confine the heat to the center of the cupola, causing a minimum heat loss in the water jacket, and a maximum melting effect in the center. This center melts rapidly and caves down as the molten slag runs into the forehearth. As the center caves the hot calcined rock, which is high on the sides, slides into the caved center and additional rock is then charged to the sides to keep them normal.

Combustion takes place in a zone or hot spot about as indicated on the drawing, Fig. 5. It is not possible to observe conditions while operating, but these conditions may be inferred from indications found upon closing down and cleaning out the cupola. There is a clinker of molten slag and unmelted rock mixed together around the burners, extending down part way on the weir and up a short distance on the nose of the inclined upper wall or arch. This condition extends rearwardly a distance of approximately two feet from the burners, under the typical conditions here described, including a gas pressure of one point per square inch at the nozzles.

It is found that the melting zone exists in an area about as indicated on Fig. 5, and extending rearwardly from the burners about twenty-four

inches, and downwardly and upwardly from a vertical line passing through the burner a maximum of twelve to fifteen inches. About this melting zone there exists a preheating and calcining zone extending upwardly from the top of that zone about two feet, and above that zone the moisture is removed by evaporation.

It has been observed on dumping that little change has taken place in the rock below the combustion or melting zone, and slag does not tend to settle to the bottom of the cupola.

In starting up, the forehearth burners 23 are lighted and fuel flow gradually increased until slagging begins before the back burners are turned on. The cupola is first charged with rock to a height of about one foot above the back burners. As the rock shows color on the surface, additional rock is charged from time to time until the charge is about six inches from the top of the water walls. In charging the cupola the fresh charge is placed next to the shell and the rock is kept twelve inches or more higher at the shell than in the center. The center core caves down and fresh rock is periodically charged to the outside as described above.

After slagging begins, the back burners are turned on and fuel pressure gradually increased to maximum fire. Between three and four hours are required to start blowing from the time the hearth burners are lighted. The operation is, of course, continuous thereafter until it is desired to close down the furnace for servicing or for other reasons.

When shutting down the furnace the charging is stopped and the rock is melted down until the fire from the back burners breaks through. The back burners are then shut off, but the forehearth burners are left on until slagging diminishes to a point unsuitable for blowing. If desired, the back and furnace burners can be shut off with the cupola full of rock, and the cupola dumped immediately, as there is very little slag in the cupola. The cupola dumps fairly clean, but there will be some scabs of slag along the inclined upper wall or arch, and along the upper part of the weir.

The problem presented, and which has been solved by this invention, is to secure a flow of slag into the forehearth without the slag carrying with it any unmelted rock, and without the rock caving or the slag flowing out of control, to cut off the slag outlet into the forehearth. This is assisted by the inclination of the walls above and below the outlet 10. It has been found that a substantial variation in the size of the opening 10, or in the lateral positioning of the weir 9 with respect to the arch 8, will ruin the results. A vertical distance of six inches, between the top of the weir 9 and the bottom of the arch 8, is correct for the size of rock and pressure of the fuel. A variation of these conditions might require a change in the size of opening. It is believed, however, that this distance is correct for ordinary operating conditions. Experience indicates that the top of the weir should be almost directly below the bottom of the arch 8. The inner surface of the lip of the weir, as well as the slot or opening 10, must be in the region of intense heat.

Melting takes place seemingly only in the combustion zone, so that this melting is the result of surface combustion on the rock, and not to any great extent as a result of radiation and convection, although as indicated, the heat from the forehearth is sufficient to start the slagging. It

is probable that heat from the forehearth assists materially in applying heat directly at the outlet 10, and in this way maintaining proper operating conditions at the outlet.

The apparatus is highly efficient both in the consumption of gas and in the utilization of space. Since the heat is applied by surface combustion, a high temperature is maintained in a restricted area to give a relatively high yield of slag.

The fact that the slag does not tend to settle to the bottom of the cupola, indicates that an unusual occurrence takes place. The viscous slag flowing over the weir tends to drag with it the molten material back out of the outlet and from below the top of the weir. The back burners apply an intense heat at these critical locations so that any rock entrained with the slag is completely melted before it passes over the weir. The drag or pull of the slag passing over the weir and falling to the bottom of the forehearth is sufficient to elevate the molten slag back of the weir to such an extent as to prevent its passing to the bottom of the cupola.

The slope of the walls above and below the opening 10 and their relative arrangement, with the arrangement of the back burner, is such as to prevent a collapse of the material in the cupola to the extent that it will block the exit, or to an extent that unmelted rock will flow over the weir with the melted slag.

As the molten slag flows over the weir 9 and cascades to the bottom of the forehearth, its viscous character serves to drag with it slag from the bottom of the melting zone although that may be considerably below the top of the weir. This dragging effect serves to bleed the molten material from the mixture of rock and slag throughout the fusion zone. While the compactness of the mass prevents displacement of the larger rocks, the particles which become entrained in the viscous fluid generally are small and are melted before passing through the opening into the forehearth, where any that do pass are fused. This bleeding action keeps the mass in the bulbous melting zone gas permeable so that the fuel mixture has access to all parts of the zone.

While the apparatus has been described as adapted for the use of gaseous fuel such as natural gas, it is to be understood that with modifications of the burners, liquid or even pulverized fuel may be employed.

It will be seen from the foregoing that the invention accomplishes its objects. Various changes may be made in the details of construction, within the scope of the appended claims, without departing from the spirit of this invention. Parts of the invention may be used to advantage without the whole, and improvements may be added while retaining the benefits of the invention.

I claim:

1. A cupola for fusing material having an opening for the discharge of fused material, said opening being formed by an upper wall or arch spaced above a bottom wall or weir, the arch being hollow to hold water, and a burner in the cupola projecting inwardly from the arch and connected through a shell of the arch to a manifold within the hollow of the arch and therein surrounded by water.

2. A cupola for fusing material having an opening for the discharge of fused material, said opening being formed by an upper wall or arch spaced above a bottom wall or weir, the interior side of the upper wall being inclined upwardly and out-

wardly from the opening, and a burner in the cupola at the opening, so positioned and directed that the area across, above and directly to the rear of the opening is a melting zone subject to heat sufficiently high to readily fuse the material.

3. A cupola for fusing material having an opening for the discharge of fused material, said opening being formed by an upper wall or arch spaced above a bottom wall or weir, the interior side of the upper wall being inclined upwardly and outwardly from the opening, the interior side of the lower wall being inclined inwardly and downwardly from the opening, and a burner in the cupola at the opening, so positioned and directed that the area across, above, below, and directly to the rear of the opening is a melting zone subjected to heat sufficiently high to readily fuse the material.

4. Apparatus for fusing material comprising a cupola having an opening for the discharge of fused material, said opening being formed by an upper wall or arch spaced above a bottom wall or weir, the interior side of the upper wall being inclined upwardly and outwardly from the opening, the interior side of the lower wall being inclined inwardly and downwardly from the opening, a burner in the cupola at the opening, so positioned and directed that the area across, above, below, and directly to the rear of the opening is a melting zone subjected to heat sufficiently high to readily fuse the material, and a forehearth communicating with the cupola through said opening having independent burners, whereby the heat therein may be regulated to produce a desired consistency of the material before discharge therefrom.

5. A cupola for fusing material having an opening for the discharge of fused material, said opening being formed by an upper wall or arch spaced above a bottom wall or weir, the interior side of the upper wall being inclined upwardly and outwardly from the opening, the interior side of the lower wall being inclined inwardly and downwardly from the opening, and a burner in the cupola at the opening, so positioned and directed that the area across, above, below, and directly to the rear of the opening is a melting zone subjected to heat sufficiently high to readily fuse the material, the opening being of a height above a floor outside the cupola sufficiently greater than the depth of the melting zone below the opening that the flow of viscous molten material in passing through the opening and falling to said floor will drag the molten material from the bottom of the melting zone.

6. In the method of fusing solid material, providing a body of raw material in a chamber, projecting a combustible mixture of air and fuel into a section of the chamber and burning the fuel upon the surface and in the interstices of the said material by surface combustion in a manner and extent to fuse progressively the material in said section, withdrawing fused material from said section and from the chamber as it is formed, thereby permitting said section to be fed with raw material by gravity, and conducting the combustion gases outwardly and upwardly from said section whereby the raw material about and above the section is preheated by convection and conduction.

7. In the method of fusing solid material, providing a body of raw material in a chamber, projecting a combustible mixture of air and fuel into a section of the chamber and burning the fuel upon the surface and in the interstices of the

said material by surface combustion in a manner and extent to fuse progressively the material in said section, withdrawing fused material from said section and from the chamber as it is formed, thereby permitting said section to be fed with raw material by gravity, conducting the combustion gases outwardly and upwardly from said section whereby the raw material about and above the section is preheated by convection and conduction, and then further conditioning the fused material to bring it to a desired temperature and consistency by subjecting it to applied heat in a second chamber.

8. In the method of fusing solid material, providing a body of raw material in a chamber, projecting a combustible mixture into a section of the chamber laterally to the rear of a restricted opening in the chamber to cause surface combustion on the material in said section in a manner and extent to fuse progressively the material in said section, bleeding fused material from said section through said opening as it is formed, thereby permitting said section to be fed with raw material by gravity, and conducting the combustion gases outwardly and upwardly from said section whereby the raw material about and above the section is preheated by convection and conduction.

9. In the method of fusing solid material, providing a body of raw material in a chamber, projecting a combustible mixture into a section of the chamber laterally to the rear of a restricted opening in the chamber to cause surface combustion on the material in said section in a manner and extent to fuse progressively the material in said section, bleeding fused material from said section through said opening as it is formed, thereby permitting said section to be fed with raw material by gravity, conducting the combustion gases outwardly and upwardly from said section whereby the raw material about and above the section is preheated by convection and conduction, and then further conditioning the fused material to bring it to a desired temperature and consistency by subjecting it to applied heat in a forehearth adjacent the fusion chamber.

10. Apparatus for fusing solid material comprising a fusion chamber adapted to be filled with raw material, a forehearth at one side of and communicating with the fusion chamber through an opening in a wall separating the fusion chamber from the forehearth, a fuel nozzle in the fusion chamber at and inwardly directed from the said opening whereby a mixture of fuel and air flowing under pressure through the nozzle will burn by surface combustion upon the surface and in the interstices of the material in the fusion chamber directly to the rear of the opening, and a separate burner in the forehearth.

11. Apparatus for fusing solid material comprising a fusion chamber adapted to be filled with raw material, a forehearth communicating with the fusion chamber through an opening in a wall separating the fusion chamber from the forehearth, a burner for heating the forehearth, a fuel nozzle in the fusion chamber at and inwardly directed from the said opening whereby a mixture of fuel and air flowing under pressure through the nozzle will burn by surface combustion upon the surface and in the interstices of the material in a melting zone in the fusion chamber directly to the rear of the opening, the opening being approximately six inches in height and substantially above the bottom of the forehearth whereby flow of viscous molten material

in flowing through the opening and falling to the floor of the forehearth will drag molten material from the melting zone in the fusion chamber.

12. Apparatus for fusing solid material comprising a fusion chamber adapted to be filled with raw material, a heated forehearth communicating with the fusion chamber through an opening in a wall separating the fusion chamber from the forehearth, and a fuel nozzle in the fusion chamber at and inwardly directed from the said opening whereby a mixture of fuel and air flowing under pressure through the nozzle will burn by surface combustion upon the surface and in the interstices of the material in a melting zone in the fusion chamber directly to the rear of the opening, the opening being of a height above the forehearth sufficiently greater than the depth of the melting zone below the opening that the flow of viscous molten material in passing through the opening and falling to the bottom of the forehearth will drag the molten material from the bottom of the melting zone.

13. A cupola for fusing solid material having an opening for the discharge of fused material, said opening being formed by an upper wall or arch spaced above a bottom wall or weir, and a fuel nozzle in the cupola at and inwardly directed from the said opening whereby a mixture of fuel and air flowing under pressure through the nozzle will burn by surface combustion upon the surface and in the interstices of the material in the cupola directly to the rear of the opening.

14. A cupola for fusing material having an opening for the discharge of the fused material, said opening being formed by an upper wall or arch spaced above a bottom wall or weir, the interior side of the upper wall being inclined upwardly and outwardly from the opening, and a plurality of nozzles in the cupola at the opening for the introduction of a gaseous component of combustion, so positioned and directed that fuel in the area across, above and directly to the rear of the opening will burn in said zone at a heat sufficiently high to readily fuse the material.

15. A cupola for fusing material having an opening for the discharge of the fused material, said opening being formed by an upper wall or arch spaced above a bottom wall or weir, the interior side of the upper wall being inclined upwardly and outwardly from the opening, a gas line for carrying oxygen, and a plurality of nozzles connected with the gas line in the cupola at the opening for the introduction of a gaseous component of combustion, so positioned and directed that fuel in the area across, above and directly to the rear of the opening will burn in said zone at a heat sufficiently high to readily fuse the material.

OLIVER J. NELSON.

#### REFERENCES CITED

The following references are of record in the file of this patent:

#### UNITED STATES PATENTS

| Number    | Name       | Date          |
|-----------|------------|---------------|
| 1,032,745 | Dow        | July 16, 1912 |
| 1,322,516 | Barnes     | Nov. 25, 1919 |
| 1,656,828 | Powell     | Jan. 17, 1928 |
| 2,057,393 | Powell     | Oct. 12, 1936 |
| 2,165,242 | Drill      | July 11, 1939 |
| 2,311,870 | Richardson | Feb. 23, 1943 |